

(No Model.)

C. VAN GÜLPEN.  
FIRE KINDLER.

No. 363,703.

Patented May 24, 1887.



Carl van Gulpén,

INVENTOR

By *Samuel R. Gaynor*

Attorney

WITNESSES

*J. Steamer*  
*Bennett S. Jones*

# UNITED STATES PATENT OFFICE.

CARL VAN GÜLPEN, OF SAN FRANCISCO, CALIFORNIA.

## FIRE-KINDLER.

SPECIFICATION forming part of Letters Patent No. 363,703, dated May 24, 1887.

Application filed September 20, 1886. Serial No. 214,010. (No specimens.)

*To all whom it may concern:*

Be it known that I, CARL VAN GÜLPEN, a citizen of the United States, and a resident of San Francisco, in the county of San Francisco and State of California, have invented certain new and useful Improvements in Fire-Kindlers; and I do hereby declare that the following is a full, clear, and exact description of the invention, which will enable others skilled in the art to which it appertains to make and use the same, reference being had to the accompanying drawing, which forms a part of this specification.

My invention has relation to fire-kindlers adapted for igniting coal and wood fires, and also for use as a fuel, if desired, and in the drawing hereto annexed I have shown a perspective view of one of my improved fire-kindlers or fire-kindling blocks, showing the shape in which I prefer to make the same.

To prepare my improved fire-kindler I use the following ingredients in proportions substantially as set forth, to wit: vegetable matter—such as the refuse from fruit-canning establishments, beet-root-sugar factories, or from vineyards and distilleries—seventy-five pounds; resin, one hundred pounds; pulverized coal mixed with charcoal, fifty pounds; brea, twenty-five pounds; tallow, twenty-five pounds; crude petroleum, about one gallon. The vegetable matter herein referred to should first be thoroughly dried, so as to remove all traces of moisture, after which it is ground and granulated in a suitable mill to a powder about as fine as sawdust. If vegetable matter or refuse of this nature is not readily obtainable, the same quantity of sawdust may be used in its place.

To prepare my improved fire-kindling blocks from the foregoing materials, I first mix the resin and tallow in proper proportions and melt the same in a suitable vessel by steam-heat. The granulated vegetable matter is thoroughly mixed and beaten up with the pulverized coal, charcoal, and brea by placing it in a revolving drum or beating-engine, or any other machine adapted for the purpose, and after these ingredients have been thoroughly mixed together they are incorporated with the mixture of melted resin and tallow in a

vessel subjected to a moderate heat, so as to keep the melted resin and tallow sufficiently fluid to cause the thorough admixture of the ingredients. Lastly, the petroleum is added, and the whole mixture is thoroughly stirred by any suitable means, so as to form a homogeneous plastic mass of such a consistency that it may readily be molded or pressed into blocks of suitable shape.

I prefer to make the blocks by pressing the material into molds by means of any suitable press, blocks thus produced being either circular or square in shape, and in size about two inches in length and in width, and about three-fourths of an inch in thickness. I do not, however, confine myself to any particular size or shape of the blocks, as that will depend in a measure upon the purposes for which they are to be used; but when they are to be used for the purpose of kindling wood or coal fires, the size above stated will be found amply sufficient, as a small block of that size or a one-inch cube will burn for a period of thirty minutes, or long enough to cause half a gallon of cold water to boil in ten minutes. In order to prevent the plastic material from sticking to the plungers of the press in which the blocks are shaped, it is advisable to let the mixture cool off considerably before it is placed in the press, or to wash the plungers occasionally with water or coal-oil. The press may be worked either by hand-power or by machinery, as may be desired.

The material known as "brea," which forms one of the ingredients in my improved fire-kindler, is a natural hydrocarbon in the nature of a natural oily or bituminous substance, which is found in large quantities in southern California. It exudes from the ground in certain localities, and after exposure to the atmosphere becomes hard and brittle. It contains a much larger percentage of bitumen than the ordinary natural asphalt, and, while admirably adapted for the purpose to which I apply it, does not seem to be as well fitted for use in pavements as the Trinidad and other natural asphalts. I have found by practical experience that the proportions of the several ingredients hereinbefore given are productive of the best results; but it is obvious that these

proportions may be varied in several respects without deviating essentially from the spirit of my invention, and I desire it to be understood, therefore, that I do not confine myself 5 to the exact proportions stated; but

What I claim, and desire to secure by Letters Patent of the United States, is—

As an improved article of manufacture, a fire-kindler adapted for use as an artificial fuel, 10 and consisting of the following ingredients: granulated vegetable matter, resin, pulverized coal mixed with charcoal, pulverized brea, tal-

low, and crude petroleum mixed in about the proportions set forth, and molded under pressure into blocks of suitable size and shape, substantially as set forth. 15

In testimony that I claim the foregoing as my own I have hereunto affixed my signature in presence of two witnesses.

CARL VAN GÜLPEN.

Witnesses:

THIREME LANDRY,  
CHAS. T. STANLEY.